

## UNITED STATES PATENT OFFICE

1,958,315

## PREPARATION OF EFFECT THREADS

Alfred Rheiner, Basel, Switzerland, assignor to  
the firm Chemical Works formerly Sandoz,  
Basel, Switzerland

No Drawing. Application July 17, 1929, Serial  
No. 379,078. In Great Britain July 24, 1928

1 Claim. (Cl. 8—20)

In the specification of the U. S. Patent No. 1,861,320, filed June 16, 1927, a process for the production of effect threads consisting of mono- or diacetate of cellulose is described. According to this specification vegetable fibres in any form (loose material, yarns, woven fabrics, in a dry, moist, raw, bleached or dyed state) are left in an acetylating mixture consisting of acetic anhydride, glacial acetic acid and one of the catalysts as usually employed for the preparation of cellulose triacetate, only until the desired mono- or diacetylation is reached. As the acetylation proceeds under emission of heat and, as the acetylating mixtures as well as the vegetable fibres are bad conductors of heat, with large charges local overheatings may occur, which might have the effect that the fibres in such places become hard and shrunk.

It has now been found that, to prevent an irregular acetylation, it is advantageous in such operation to keep the acetylation mixture or the fibres in movement. This precautionary measure is especially necessary, when threads in package form such as cops, cakes, cheeses, warp threads 25 wound on beams and the like, are to be treated.

The circulation of the acetylating mixture or the movement of the fibres in this mixture does not only prevent an irregular acetylation, but it further results in different unexpected advantages.

The acetylation under circulation of the mixture can for instance be carried out at a much higher temperature, without increasing the risk of obtaining uneven results; this is especially desirable, if mixtures containing smaller quantities of acetic anhydride, are employed. The working with these mixtures is of a considerable economic importance. Acetic anhydride being the most expensive constituent of the mixture, it is obvious that the acetylation process becomes cheaper with mixtures containing as little anhydride as possible. Up to the present the working with such mixtures was considered to be impossible as well as the process described in the aforesaid specification (see Hottenroth, Die Kunstseide 1926, page 354, lines 13-22). Contrary to this opinion it has been found that for instance cellulose monoacetate can be produced without difficulty with mixtures containing no more than the 45 theoretically required quantity of acetic anhydride, if the acetylation is effected at a somewhat increased temperature and whilst keeping the fibres in movement; furthermore the threads thus obtained possess an extraordinarily soft 55 touch.

The acetylation in the above described manner can also be carried out with great advantage, if the cellulose material, instead of immersing same in an acetylation mixture consisting of acetic anhydride, glacial acetic acid and a catalyst, is first treated with one or two of the constituents of the mixture and the remaining constituent or constituents are subsequently added. The cellulose material can thus first be placed in glacial acetic acid and the acetic anhydride and the catalysts 60 added later, or it can first be impregnated with acetic anhydride and glacial acetic acid and the catalyst added later. Moreover, the cellulose may first be impregnated with the catalyst and the acetic anhydride and the glacial acetic acid 65 added later, or the fibres, which have been impregnated with the catalyst, are introduced into a bath containing the mixture of acetic anhydride and glacial acetic acid.

Still other variations consist in introducing the 75 cellulose material into a mixture of acetic anhydride and glacial acetic acid and adding the catalyst later or in introducing the cellulose fibres first either into a mixture of glacial acetic acid or of acetic anhydride and the catalyst and adding the acetic anhydride, respectively the glacial acetic acid later.

Each of these methods can afford satisfactory results when combined with suitable conditions of reaction. The circulation of the mixture is of 85 great advantage as it allows of a quick mixing of the liquor and consequently of a uniform action on the fibres.

The following examples illustrate the improved process, the parts being by weight.

*Example 1*

100 parts of kier-boiled cotton yarn are introduced into an acetylating mixture consisting of 30 parts of zinc chloride, 100 parts of acetic anhydride and 870 parts of glacial acetic acid of 100% strength. The material is treated at 60° C. for about 10 hours whilst keeping the liquor in continuous circulation by means of a pump. Thereupon the yarn, which is unaltered in its structure, is taken out and separated from the mixture as completely as possible, washed and dried. The effect threads produced in this way remain practically uncolored in a dyebath containing substantive colours reserving acetate silk.

100

105

*Example 2*

100 parts of bleached, dried cotton yarn are introduced into an acetylating mixture consisting of 40 parts of zinc chloride, 80 parts of acetic 110

anhydride and 880 parts of glacial acetic acid of 100% strength, so that the yarn is completely covered by the liquid. The bath is kept in regular circulation for 12 hours, whilst maintaining its temperature at 50° C. Thereafter the yarn is hydroextracted, washed and dried. 125 parts of a treated yarn are obtained, hardly distinguishable from the initial material as regards appearance, but which has no affinity at all for substantive dyestuffs.

*Example 3*

100 parts of bleached cotton yarn are brought into a closed vessel. Ten times its weight of a warm acetylating mixture containing 5% of zinc chloride, 15% of acetic anhydride and 80% of glacial acetic acid of 100% strength, are pumped therethrough for 3/4 hour at 80° C. The yarn is then freed from the acetylating mixture as completely as possible, immersed in ice-water, well rinsed, soaped and dried. The effect threads thus prepared are completely refractory to dyeing with suitable substantive dyestuffs.

*Example 4*

100 parts of raw cotton yarn are introduced into a bath of 700 parts of 98% glacial acetic acid. After a short time 250 parts of acetic anhydride and 50 parts of zinc chloride are added and the liquid kept in movement, at a temperature of 40° C., until a test, after washing and drying, can no longer be dyed with 1% Chloramine Sky blue FF (Colour Index of Dyers and Colorists, Bradford 1924, 1st edition, No. 518), which is the case after about 24 hours. Thereupon the yarn is separated from the liquor, washed and dried.

*Example 5*

100 parts of cops dyed with Sulphur black T (said Colour Index, No. 978) and freed from any moisture are brought into a suitable vessel containing 800 parts of a mixture consisting of 10% of acetic anhydride, 3% of zinc chloride and 87% of glacial acetic acid 100%. After pumping through for 8 hours at 60° C. the cops are hydroextracted, washed and dried. The black effect

threads thus prepared keep, in cross-dyeing with substantive dyestuffs, their deep black shade.

*Example 6*

Cotton yarn dyed with Indanthrene blue GCD (said Colour Index, No. 1113) is transformed into dyed cellulose monoacetate by one of the processes described in the preceding examples. Although the glacial acetic acid is an excellent solvent for vat dyestuffs, the acetylating mixtures remain in spite of the continuous circulation, practically undyed.

The foregoing examples illustrate the use of zinc chloride as catalyst. Obviously any other catalyst used for the production of cellulose acetate, such as halogen hydroacids, nitric acid, phosphoric acid, halogenated fatty acids etc. may be employed whilst choosing the appropriate conditions of reaction.

What I claim is:

A process for the preparation of effect threads, having no affinity for substantive dyestuffs and consisting of the lower acetylated derivatives of cellulose by the direct acetylation of cellulosic fibres without altering the original structure of such fibres, the reaction being effected in a single bath and in a single operation by immersing natural cellulosic fibres in any form in an excess of an acetylating mixture maintained at a temperature between approximately 40° and 80° C. and consisting of acetic anhydride, glacial acetic acid and an acetylating catalyst, the fibres being entirely covered by and in contact with excess of acetylating mixture throughout the course of the reaction and allowing the acetylating mixture to react on the fibres only until the mono- and diacetyl derivatives of cellulose have been formed, thereupon separating the resultant effect threads from the excess of acetylating mixture, said process being characterized in that the acetylating mixture does not contain more acetic anhydride than is theoretically necessary for the production of mono- and diacetyl derivatives of cellulose and in that during the acetylating operation a continuous relative movement is produced between the acetylating mixture and the cellulose fibres.

ALFRED RHEINER.

50

125

55

130

60

135

65

140

70

145

75

150